

W. A. HALL.

PROCESS OF PREVENTING THE ESCAPE OF SULFUR DIOXID IN SMELTING SULFID ORES.  
APPLICATION FILED JUNE 30, 1913. RENEWED MAR. 1, 1915.

1,134,846.

Patented Apr. 6, 1915.



Witnesses:

C. M. Sweeny  
M. E. Patterson

Inventor:

William A. Hall,

By *Albert Ralston*

Attorneys

# UNITED STATES PATENT OFFICE.

WILLIAM A. HALL, OF NEW YORK, N. Y.

## PROCESS OF PREVENTING THE ESCAPE OF SULFUR DIOXID IN SMELTING SULFID ORES.

1,134,846.

Specification of Letters Patent.

Patented Apr. 6, 1915.

Application filed June 30, 1913, Serial No. 776,620. Renewed March 1, 1915. Serial No. 11,328.

*To all whom it may concern:*

Be it known that I, WILLIAM A. HALL, citizen of the United States, residing at New York, in the county of New York and State of New York, have invented or discovered certain new and useful Improvements in Processes of Preventing the Escape of Sulfur Dioxid in Smelting Sulfid Ores, of which the following is a specification, reference being had therein to the accompanying drawing.

The object of the present invention is to overcome the nuisance created by the discharge of sulfurous gases from furnaces in which sulfid ores are smelted, by the conversion of the bulk of the  $\text{SO}_2$  present into free sulfur, and, if desired, the subsequent separation and recovery of this elemental sulfur from the exit gases, in a commercial form, thereby obtaining a valuable by-product.

The present invention relates to a process for the recovery in elemental and commercial form of the sulfur evolved from pyrites in the operation of smelting copper in the well known water jacketed pyritic smelters used for the purpose, and for preventing the discharge of noxious sulfur dioxid fumes from the furnace into the atmosphere.

In the manner in which the operation of pyritic smelting is at present conducted the only portion of the sulfur that is of use as fuel is that portion commonly known as the non-volatile which is below the pyrrhotite ( $\text{Fe}_6\text{S}_7$ ) state (generally considered as the Fe, FeS state). All the sulfur content of the pyrites above this Fe, FeS state, that is to say all of the volatile sulfur and a part of the non-volatile sulfur is separated from the pyrites and discharged without being of any use as a fuel in assisting the operation. At a certain zone in the furnace this separated portion of the sulfur exists in the furnace gases in an elemental condition, in the form of heavy sulfur fumes. This zone is approximately about  $2\frac{1}{2}$  ft. above the slag forming nucleus, or  $5\frac{1}{2}$  ft. above the twyers and perhaps 7 to 8 ft. below the top of the charge. Higher up in the furnace at or near the top of the charge where it meets with atmospheric air, this sulfur vapor burns fiercely to  $\text{SO}_2$ . Could the current of fumes and gases issuing from the top of the furnace be hermetically sealed against the outer air, then this volatile sul-

fur would pass off in the elemental state and could be collected, but this has heretofore never been accomplished owing to the necessity of giving a free discharge of the air blown in through the twyers and consequent products of combustion. Often from 5000 to 10000 cubic feet of air is blown in per minute, and this is greatly increased in volume within the furnace owing to its expansion upon heating to the temperature in the focus. If this air and products of combustion were not given a most free vent, the operation of the furnace would be checked. In any case there is naturally a great inrush of air accompanying the feeding in of the pyrites charge.

If the hermetic sealing were possible, the discharge would contain much sulfur dioxid from the combustion taking place in the lower portion of the furnace, and although a certain portion of sulfur could be recovered, the sulfur vapor would be contaminated by the presence of much sulfur dioxid which in itself would be a great nuisance if permitted to escape into the outer air. Furthermore there would be lost a considerable sulfur value in this sulfur dioxid. In accordance with the present invention I condense and recover substantially all of this sulfur *i. e.* both that existing as elemental sulfur, that existing as  $\text{SO}_2$ , in the gases and this I may accomplish by admitting a reducing flame, preferably with steam, into the upper level of the furnace. In case a furnace having a hermetically sealed head is used, there is not sufficient inrush of false air, at the top of the furnace to do any great harm. Moreover enough internal pressure is created in the furnace, by the expansion of the air blown in through the twyers, and the gases evolved in the decomposition of the pyrites, to prevent the above mentioned inrush of air, even if the reducing flame is not blown in at the upper level, but the sulfur already existing as  $\text{SO}_2$  would be lost. By passing the products of combustion carrying the elemental sulfur in suspension through separating devices hereinafter described, I can recover the sulfur. This reducing gas can be water gas or air and water gas obtained from a gas producer and containing much carbon monoxid and hydrogen, although other varieties of gas can be used. This gas flame serves a three-fold purpose: (1) it prevents oxidation of the sulfur vapor, (2) it

it reduces the sulfur dioxid to sulfur and (3) it imparts a desirable high temperature at the upper level of the furnace necessary to bring about this reduction, as the sulfur dioxid cannot be deoxidized by reduction excepting at very much higher temperatures than exist normally in the upper portion of the furnace. This reducing gas may be admitted at about the normal level of the pyritic charge, thereby preventing the contact of free air with the top of the charge, but if desired may be introduced at a lower level. Also under certain conditions, such as the employment of a reducing gas poor 10 in hydrogen, it is found desirable to admit along with the reducing gas a certain amount of steam or water vapor in order to produce a certain amount of sulfureted hydrogen, which is a practical agent for 15 decomposing the sulfur dioxid present, said steam also decomposing any carbon oxysulfid (COS) that may be formed, but I do not care to limit myself to the use of this steam for under certain conditions (as for 20 instance where a little sulfur dioxid may be allowed to escape) it may not be found necessary. The sulfur then contained in the 25 gases leaving the upper part of the furnace is all, or substantially all, in the condition 30 of elemental sulfur and can be readily separated from the nitrogen, carbon dioxid and other products of combustion by any suitable means, as for instance by passing the entire volume of fumes through a gas 35 washer or condenser of the well known Heisen type or any other suitable gas washer designed specially for the extraction of solid and sticky matter from furnace gases. Such a device can be operated in a 40 manner to create no back pressure on the furnace.

One difference between the present invention and those described in my copending applications 725,024, filed Oct. 10, 1912; 45 770,946, filed May 31, 1913, and 773,456, filed June 13, 1913, which cases also show and claim the treatment of sulfid ores with a reducing flame, is this that in the present case the reducing flame is not primarily used 50 for decomposition of the pyrites *i. e.* the separation of the bulk of the sulfur from the pyrites or other ore and its volatilization are not effected by the reducing flame, but are effected primarily by the temperature im- 55 parted to the ore charge by combustion of sulfur and iron at the fusion zone, sending up hot products of combustion of more or less neutral character (neutral here meaning not strongly oxidizing and not strongly re- 60 ducing). The reducing flame, however, does decompose the sulfur dioxid present and may volatilize some of the sulfur of the pyrites, and may produce some H<sub>2</sub>S, the latter either from the action of steam on the hot

pyrites, or by the action of the hydrogen of 65 the gas on the pyrites. Also the stable equivalent for the bulk of the iron in the present case is not nascent oxygen obtained from the decomposition of water, but is atmospheric oxygen from the air admitted through the 70 twyers and the silica of the quartz which is always used in pyritic smelting.

The preferred temperature to be maintained by the reducing flames at the top of the ore charge may be stated as about 700° 75 C., or a little over. It is obvious that the ore must not be heated to 900° C., or over, since it would then become molten, and any amount of melting would cause it to sinter, and cause trouble. 80

The process may be carried out in a furnace as shown by way of example in the accompanying drawings, in which a modified structure of the ordinary water-jacketed pyritic smelter is illustrated. 85

In said drawing the charge is admitted through the doors 1, or in any other suitable manner, which doors should be capable of being tightly closed when ore is not being charged into the furnace. The air for the combustion of the sulfur of the ore is admitted through suitable twyers 2, connected with a belly pipe 3, in the usual manner, the charge of ore in the lower part of the furnace is maintained at the usual smelting temperature, and the gases ascending through the charge contain free sulfur, some SO<sub>2</sub> and CO<sub>2</sub>, and a large amount of free nitrogen, and are drawn off in the usual manner through the pipe 4, to which is connected a flue 5, carrying the gases to a gas washer, of any approved type. A stack 6 may also be provided for allowing the entire fumes and gases to pass into the atmosphere, should the gas washer become temporarily 90 clogged up, or should repairs be necessary to the gas washer. This part of the process is all well known and old, and does not need any elaborate description here. 95

The line 7 of the drawing represents what 100 may be termed the "normal level" of the charge of ore and flux in the furnace, although this will vary more or less, and may at times be considerably above the blast lamps to be now referred to. 110

Slightly above the normal charge level of the furnace charge I provide suitable blast lamps 8 which I connect with a supply of air and gas 9 and 10 respectively, through which I introduce a reducing flame, for accomplishing the purposes above referred to. If desired steam may also be introduced through either the pipe 9 or 10, along with the gas or air, or through a pipe 11, suitably connected with one or more of these blast 120 lamps, or may be supplied to the furnace by independent pipes, but as stated above the introduction of steam is to some extent op- 125

tional, and in using steam I preferably use a small amount only. If desired some of the blast twyers 8 may be used for admitting gas alone, without any air, should it be found that quite large amounts of false air are entering through the charging doors, or otherwise. I may also prevent the entrance of false air to a very large extent, by allowing the gases in the smelter to be under more or less pressure.

The reduction of the  $\text{SO}_2$  may or may not be completed within the furnace itself. In case material amounts of steam are used with the reducing flame some  $\text{H}_2\text{S}$  is formed, which will travel along with the gases still containing  $\text{SO}_2$ , and the reaction between these two will take place after the temperature has fallen somewhat, which will be outside the furnace itself, but before the gases reach the gas washer. In case the reducing flame does not contain much hydrogen and an insufficient amount of steam is introduced with the flames, considerable  $\text{COS}$  may be formed, which will be acted upon by steam introduced into the exhaust flue leading to the gas washer, said steam decomposing the  $\text{COS}$ , according to the reaction



which  $\text{H}_2\text{S}$  will reduce any  $\text{SO}_2$  still present in the gases, in accordance with the reaction



Accordingly it is advisable to carefully regulate the reducing flames for the complete ultimate reduction of all the  $\text{SO}_2$ , without leaving material amounts of  $\text{H}_2\text{S}$  in the gases leaving the washer.

In all places in the process where steam is referred to, it is obvious that water, in suitable amount could be used, since the temperatures are such as to convert such water into steam, and the use of the term "steam" in the appended claims is intended to cover the use of water or any material which would be the equivalent, such as aqueous solutions.

I disclaim the treatment of the gases, after leaving the smelting furnace, with reducing gases, or with a bed of coke or the like, for the recovery of sulfur therefrom. In my process, a considerable portion of the sulfur comes upwardly through ore charge as elemental sulfur and never becomes oxidized to sulfur dioxid, either in or out of the smelting furnace. The treatment of the ore and the gases, for the reduction, all takes place in my process within the furnace itself.

What I claim is:—

1. A process of recovering elemental sulfur in smelting sulfid ore, and for preventing the escape of noxious gases, which com-

prises introducing a reducing gas flame, into the upper level of the furnace, at a point near the normal charge level therein, said flame being capable of reducing a part at least of the sulfur dioxid to elemental sulfur, while preventing the access of sufficient air to the gases leaving the smelting furnace to oxidize any considerable quantity of the elemental sulfur existing in, or produced in said gases, until the temperature of said gases has fallen below the temperature at which free sulfur will oxidize, and separating the elemental sulfur from said gases.

2. A process of recovering elemental sulfur in smelting pyritic ores, and for preventing the escape of noxious gases, which comprises introducing a reducing gas flame together with steam, into the upper level of the furnace, at a point near the normal charge level therein and under conditions capable of reducing a part at least of the  $\text{SO}_2$  in the exit gases, and thereafter separating the elemental sulfur from the gases.

3. A process of preventing the escape of noxious gases in smelting, which comprises the subjecting an upper layer of the sulfid ore charge, to the action of a reducing gas, while at a high temperature, and avoiding the presence of sufficient free air at that point to reoxidize the elemental sulfur.

4. In smelting sulfid ores, the step of preventing the escape of sulfur dioxid which comprises reducing the same, by the introduction of reducing gases, into the upper part of furnace at a point materially above the focus, and while avoiding the presence, at that point, of sufficient free oxygen to reoxidize said reduced sulfur.

5. In smelting sulfid ore, the step of introducing a reducing flame into the furnace, at a point near the normal charge level therein for reducing sulfur dioxid, and while avoiding the presence, at that point, of sufficient free oxygen to reoxidize said reduced sulfur.

6. In smelting sulfid ore, the step of introducing a reducing flame, together with steam, into the furnace, at a point near the normal charge level therein at which point an excess of sulfur dioxid is present, for reducing a part at least of said sulfur, and while avoiding the presence of substantial quantities of free oxygen at that point.

7. In smelting sulfid ores, the step of introducing a reducing flame into the furnace, at a point near the normal charge level therein, for reducing the sulfur dioxid and introducing steam into the gases and fumes leaving the furnace.

8. In smelting sulfid ores, the step of subjecting the upper layer of the ore charge, to the substantially continuous action of a reducing flame.

9. A process which comprises smelting a sulfid ore charge in a blast of air, while pre-

venting free access of the top of the ore charge to the action of air, and while subjecting an upper layer of said ore charge, to the action of a reducing flame, capable of 5 reducing at least the major portion of the sulfur dioxid therein, into elemental sulfur.

In testimony whereof I have affixed my signature, in presence of two witnesses.

WILLIAM A. HALL.

Witnesses:

A. B. FOSTER,  
A. M. PERKINS